

## UNITED STATES PATENT OFFICE

2,408,385

## DRILL LUBRICANT

Edmund L. Flood, San Diego, Calif., assignor to  
 Consolidated Vultee Aircraft Corporation, San  
 Diego, Calif., a corporation of Delaware

No Drawing. Application April 16, 1945.  
 Serial No. 588,733

9 Claims. (Cl. 252—41)

1

This invention relates to lubricants for drills of the portable and stationary types which are used to drill holes through metal, and more particularly to a sodium base grease lubricant composition which is especially adapted for use in high speed hand drilling operations in the manufacture of aircraft.

In the high speed hand drilling of metals in the aircraft industry, particularly aluminum alloys such as duralumin, there has been up to the present time a pressing need for a lubricant which will stay on the drill during rotation thereof and remain stable during the vigorous mechanical agitation and high temperature conditions to which such lubricants are subjected during drilling operations. The lubricants heretofore used in these operations are objectionable because they either fly off the revolving drill, leaving insufficient lubricant on the drill and soiling everything on which the flying lubricant settles, or are unable properly to lubricate the drill during operation because they disintegrate under the high temperature conditions generated by the drilling operation. Not infrequently, with such prior art lubricants, it was found that the duralumin welded to the revolving drill point, resulting in imperfect drillings and in the need to discard costly drills long before the useful life thereof had been fully utilized.

The lubricant composition of the present invention overcomes the foregoing defects inherent in the prior art lubricants used in high speed drilling operations and, additionally, makes possible the drilling of perfect holes through superimposed sheets of duralumin and other metals without elongation of the hole in the outer sheet. Also, it maintains the temperature generated during drilling lower than heretofore, by as much as 25% and even more, thereby prolonging the life and productivity of the drill. The lubricant composition of my invention has other advantages which will be made apparent in the following description of the composition.

The drill lubricant composition of my invention comprises a soda base grease, turpentine, a relatively high melting point wax, preferably a petroleum wax, and aluminum stearate. The proportions of the constituents of my composition are critical in that any substantial variation from the proportions set forth in the preferred illustrative embodiment set forth below will impair the effectiveness of the composition as a drill lubricant. In general, on a weight basis, the soda base grease may vary from about 45 to 52% of the composition, the turpentine from 8 to 12%,

2

the wax from 38 to 43%, and the aluminum stearate from 0.25 to 0.5%.

The soda base grease may be produced by suspending or dissolving sodium soap produced from vegetable or animal oils or fats or fatty acids in a mineral oil. Thus, this grease may be formed by incorporating into a suitable mineral oil, preferably one having high flash and fire points, a desired percentage, say about 15 to 50%, of the sodium soap of tallow, stearic acid, hydrogenated fatty acids or the like or the sodium soap of any mixture of soap forming stocks. The most effective soda base grease is one produced by incorporating from about 15 to 23% of a sodium base soap, based on the weight of the grease, in a high viscosity lubricating oil or a mixture of such oils which contain dissolved or suspended therein in a small amount, say 1 to 1.4%, of petrolatum. The preferred lubricating oil is petroleum Bright Stock alone or in combination with a mineral lubricating oil having a viscosity of 550 seconds, Saybolt, at 100° F.

The relatively high melting point wax of the composition of my invention is paraffin wax having a melting point higher than the melting points of the typical varieties of paraffin wax commercially available. Thus, the paraffin wax may have a melting point of about 143° to 170° F., preferably 160° to 165° F. Other waxes having melting points above about 143° F. such as carnauba wax, ceresin wax, candelilla wax and the like may be used, but better results are obtained with paraffin wax.

The following is an example of a preferred drill lubricant in accordance with my invention and of the method of making it. In the example, the term "parts" indicates parts by weight.

|                                     | Parts |
|-------------------------------------|-------|
| Soda base grease (17% soap content) | 50    |
| Paraffin wax, 165° F. melting point | 43    |
| Turpentine                          | 10.4  |
| Aluminum stearate                   | 0.42  |

The soda base grease, turpentine and aluminum stearate are mixed at room temperature, then heated to about 165° F. and then thoroughly mixed with the paraffin wax while the latter is in the melted state. The mixture, while still hot, is poured into a container and permitted to cool and solidify.

The grease of my composition serves as a vehicle for the turpentine, the cutting oil, and acts to give a smooth finish to the walls of the hole being drilled. The relatively high percentage of mineral oil in the soda base grease serves as an

excellent heat conductor and makes possible the drilling through metal at temperatures lower than heretofore. The relatively large amount of relatively high melting point wax of my composition serves to maintain the drill lubricant in a solidified state and prevents the oil and turpentine from draining therefrom. The aluminum stearate aids in making the composition uniform and stable and imparts film strength to the mineral oil, thereby augmenting the anti-welding properties of the lubricant composition and making possible the drilling through metal of sharp, clean holes without welding of chips or turnings to the drill point.

The herein described lubricant effectively and efficiently fulfills its intended purpose and may be applied to a drill in any suitable manner such as, for example, by inserting the drill into a closed cardboard container filled with the lubricant.

I claim:

1. A drill lubricant composition comprising, on a weight basis, from 45 to 52% of a soda base grease, 38 to 43% of paraffin wax having a melting point of at least about 143° F., 8 to 12% of turpentine and 0.25 to 0.5% of aluminum stearate.

2. The drill lubricant of claim 1 wherein the soda base grease comprises, on a weight basis, from 15 to 23% of a sodium base soap.

3. The drill lubricant of claim 1 wherein the soda base grease comprises, on a weight basis, from 15 to 23% of a sodium base soap and from 1 to 1.4% of petrolatum.

4. The drill lubricant of claim 1 wherein the soda base grease comprises, on a weight basis, from 15 to 23% of a sodium base soap, the balance being petroleum Bright Stock and 550 viscosity lubricating oil, together with about 1 to 1.4% of petrolatum.

5. A drill lubricant composition consisting of, on an approximate weight basis, 50 parts of soda base grease, 43 parts of paraffin wax having a melting point of about 165° F., 10.4 parts of turpentine and 0.42 part of aluminum stearate.

6. The drill lubricant of claim 5 wherein the soda base grease comprises, on an approximate weight basis, 17% of soda base soap and in excess of 80% of a high-viscosity lubricating oil.

7. The drill lubricant of claim 5 wherein the soda base grease comprises, on an approximate weight basis, 17% of soda base soap and in excess of 80% of a high-viscosity lubricating oil consisting of petroleum Bright Stock and 550 viscosity lubricating oil.

8. The drill lubricant of claim 1 wherein the soda base grease comprises, on a weight basis, from 15 to 23% of a sodium base soap suspended in a vehicle consisting essentially of petroleum Bright Stock and 550 viscosity lubricating oil.

9. The drill lubricant of claim 1 wherein the soda base grease comprises, on a weight basis, from 15 to 23% of a sodium base soap suspended in a vehicle consisting essentially of a high-viscosity lubricating oil.

EDMUND L. FLOOD.